

1

2,892,702

## HARDENABLE STAINLESS STEEL

Carl S. Walton, Sewickley, and William F. White, White-hall Borough, Pa., assignors to United States Steel Corporation, a corporation of New Jersey

No Drawing. Application January 4, 1955  
Serial No. 479,855

3 Claims. (Cl. 75—124)

This invention relates to improvements in the art of precipitation hardening steels of the so-called "stainless" type.

It has heretofore been proposed by Foley in Patent No. 1,943,595 to form chromium-nickel stainless steels having the chromium and nickel proportioned to form a structure which is unstably austenitic and include therein a precipitation hardening element such as aluminum so that the steel can be hardened by suitable heat treatments. However, the usefulness of such steels has been lowered considerably by the lack of uniform response to the hardening treatments and by reason of its having a tendency to partially transform after solution annealing. We have discovered that the addition of nitrogen within certain limits to steels of such type will prevent hardening following solution annealing and render the same uniformly responsive to transforming and precipitation hardening treatments.

The teachings of our invention are applicable to chromium-nickel stainless steels containing nickel in quantities insufficient to render the same stably austenitic and which can be transformed and hardened by thermal treatment.

The preferred steel of our invention which has a desirable combination of corrosion resistance and mechanical properties and which at the same time will not transform following solution annealing is uniformly responsive to transformation and aging treatments has the following preferred composition ranges:

|            | Percent        | Heat No. | C    | Mn   | P     | S     | Si   | Ni   | Cr    | Al   | N     |
|------------|----------------|----------|------|------|-------|-------|------|------|-------|------|-------|
| Carbon     | .05 to .08     | 45       | 0.05 | 1.40 | 0.015 | 0.021 | 0.58 | 5.61 | 16.44 | 1.75 | 0.12  |
| Manganese  | max. 1.5       | 2        | 0.05 | 1.38 | 0.008 | 0.020 | 0.60 | 5.67 | 16.38 | 1.27 | 0.034 |
| Silicon    | max. 1.00      | 3        | 0.08 | 1.45 | 0.008 | 0.019 | 0.59 | 6.73 | 17.40 | 0.76 | 0.17  |
| Chromium   | 16.00 to 17.50 | 4        | 0.05 | 1.21 |       |       | 0.51 | 6.36 | 16.54 | 1.14 | 0.15  |
| Nickel     | 5.50 to 6.75   | 5        | 0.08 | 1.36 | 0.008 | 0.019 | 0.57 | 6.85 | 17.56 | 0.67 | 0.17  |
| Aluminum   | .90 to 1.80    | 6        | 0.05 | 1.46 | 0.015 | 0.020 | 0.60 | 5.40 | 16.18 | 1.63 | 0.10  |
| Nitrogen   | .12 to .18     |          |      |      |       |       |      |      |       |      |       |
| Phosphorus | max. .04       |          |      |      |       |       |      |      |       |      |       |
| Sulphur    | max. .04       |          |      |      |       |       |      |      |       |      |       |

with the remainder iron and residual amounts of other elements.

In the absence of nitrogen, such an alloy will at times respond to transformation and aging treatments. However, the response varies widely for reasons unknown and frequently the steel hardens to above 95 R<sub>b</sub> following solution annealing and cooling. This has materially affected the usefulness of these steels since many heats had to be diverted to other uses. We have discovered that the addition of nitrogen in suitable amounts will prevent such hardening after solution annealing and will provide a steel which will have hardness value of less than 95 R<sub>b</sub> after solution annealing and air cooling. The nitrogen may be added by any conventional method, such as by the addition of ferro-chromium containing high nitrogen to the liquid steel melt. With our pre-

2

ferred analysis containing .12 and .18% nitrogen, after solution annealing, the steel can be treated either by heating and air cooling to transform it or by cooling to a low temperature. Heretofore, it has been necessary to vary the composition dependent on whether it was desired to transform the steel by heat treatment or by cooling to sub-zero temperatures. Following transformation our steel can be aged to a hardness in excess of 38 R<sub>c</sub>.

10 Steels having a composition within the foregoing ranges can be suitably solution annealed by heating to a temperature between 1800 and 2000° F. for sufficient time to permit the carbides to go into solution. A preferred treatment is holding for 30 minutes at 1850° F. Following this they can be air cooled to room temperature with substantially no hardening or transformation taking place and will have a hardness value less than 95 R<sub>b</sub>. Since the steel in such condition is quite soft and ductile, it can be readily formed and worked. After forming or fabrication, the steel can be transformed by either holding at a temperature below about —50° F. for sufficient time to cause the austenite to transform to martensite or by holding for sufficient time at a temperature between 1300 and 1500° F. to raise the M<sub>s</sub> point sufficiently to permit the steel to transform on cooling to room temperature. A preferred low temperature treatment is to hold for one hour at —110° F. and a preferred heat treatment is to hold it for about two hours at 1400° F.

20 30 The steel can then be further hardened to a value above 38 R<sub>c</sub> by an aging treatment which may vary considerably over a temperature range of 700° to 1100° F. At the lower temperatures considerably longer times are required but a suitable treatment is about 30 minutes at 900° F.

25 Hardness values following solution annealing, transforming and aging of the heats set forth in Table I will amply demonstrate the teachings of our invention:

30

Table I

| Heat No. | C    | Mn   | P     | S     | Si   | Ni   | Cr    | Al   | N     |
|----------|------|------|-------|-------|------|------|-------|------|-------|
| 45 1     | 0.05 | 1.40 | 0.015 | 0.021 | 0.58 | 5.61 | 16.44 | 1.75 | 0.12  |
| 2        | 0.05 | 1.38 | 0.008 | 0.020 | 0.60 | 5.67 | 16.38 | 1.27 | 0.034 |
| 3        | 0.08 | 1.45 | 0.008 | 0.019 | 0.59 | 6.73 | 17.40 | 0.76 | 0.17  |
| 4        | 0.05 | 1.21 |       |       | 0.51 | 6.36 | 16.54 | 1.14 | 0.15  |
| 5        | 0.08 | 1.36 | 0.008 | 0.019 | 0.57 | 6.85 | 17.56 | 0.67 | 0.17  |
| 6        | 0.05 | 1.46 | 0.015 | 0.020 | 0.60 | 5.40 | 16.18 | 1.63 | 0.10  |

50 55 The hardness values following solution annealing, transforming and aging of the foregoing heats are given in the following Table II, wherein all hardness values are Rockwell "C" unless otherwise specified.

Table II

| Heat No. | 30 Min. at 1,850° F.<br>Air Cool to R.T. | Transformation Treatment |                     | Transformation+Aging Treatment         |                                          |
|----------|------------------------------------------|--------------------------|---------------------|----------------------------------------|------------------------------------------|
|          |                                          | 1 Hr. at —110° F.        | 2 Hrs. at 1,400° F. | 1 Hr. at —110° F. + 30 Min. at 900° F. | 2 Hrs. at 1,400° F. + 30 Min. at 900° F. |
| 60 1     | 1 97.0                                   | 38.7                     | 33.0                | 42.5                                   | 43.0                                     |
| 2        | 30.3                                     | 35.2                     | 32.7                | 46.0                                   | 43.6                                     |
| 3        | 1 81.7                                   | 1 84.7                   | 24.0                | 1 85.2                                 | 37.5                                     |
| 4        | 1 93.0                                   | 38.0                     | 32.0                | 43.8                                   | 44.0                                     |
| 5        | 1 81.0                                   | 1 82.0                   | 1 89.5              | 1 82.0                                 | 1 92.2                                   |
| 6        | 25.0                                     | 39.2                     | 32.7                | 42.7                                   | 43.2                                     |

1 Rockwell "B."

70 75 Heat No. 1 containing .12% nitrogen was soft as annealed and could be hardened to a minimum hardness

value of 38 R<sub>c</sub> by both transformation treatments, whereas Heat No. 2 containing only 0.034% nitrogen exhibited a high hardness after annealing.

Heat No. 3 having an aluminum content below the preferred range did not harden upon aging to the specified minimum.

Heat No. 4 containing .15% nitrogen reacted much like Heat No. 1.

Heat No. 5 with three elements slightly outside the preferred range did not transform and thus could not be hardened the desired amount.

Heat No. 6 with two elements outside the range on the side of high M<sub>s</sub> temperature showed considerable transformation on annealing and thus was not satisfactory.

The steels of our invention are further characterized by an elongation of about 8% and a Charpy V notch impact value of at least 5 ft. lbs. when heat treated to a hardness value of R<sub>c</sub> 41 and a corresponding tensile strength of 165,000 p.s.i.

While we have shown and described several specific embodiments of our invention, it will be understood that these embodiments are merely for the purpose of illustration and description and that various other forms may be devised within the scope of our invention, as defined in the appended claims.

We claim:

1. A stainless steel characterized by a hardness value of less than 95 R<sub>b</sub> after solution annealing and air cooling and susceptible to phase transformation and age-hardening by double thermal treatment to a hardness value of at least R<sub>c</sub> 38 containing between .05 and .08% carbon, 16.0 to 17.5% chromium, 5.50 to 6.75% nickel, .90 to 1.80% aluminum, .12 to .18% nitrogen and the balance iron and other elements in amounts which do not adversely affect the properties.

35

2. A stainless steel characterized by a hardness value of less than 95 R<sub>b</sub> after solution annealing and air cooling and susceptible to phase transformation and age-hardening by double thermal treatment to a hardness value of at least R<sub>c</sub> 38, said steel containing between .05 and .08% carbon, 1.5% maximum manganese, 1.00% maximum silicon, 16.0 to 17.5% chromium, 5.50 to 6.75% nickel, .90 to 1.80% aluminum, .12 to .18% nitrogen with the balance iron and residual amounts of other elements.

3. Age-hardened substantially martensitic stainless steel having a hardness in excess of 38 R<sub>c</sub> characterized by initially having a substantially austenitic structure following solution annealing and air cooling and a hardness in said condition of less than 98 R<sub>b</sub>, said steel having been transformed to a martensitic structure by thermal treatment and thereafter age hardened, said steel containing between .05 and .08% carbon, 16.0 to 17.5% chromium, 5.50 to 6.75% nickel, .90 to 1.80% aluminum, .12 to .18% nitrogen and the balance iron and other elements in amounts which do not adversely affect the properties.

#### References Cited in the file of this patent

#### UNITED STATES PATENTS

|           |                |               |
|-----------|----------------|---------------|
| 2,489,520 | Camras         | Nov. 29, 1949 |
| 2,505,763 | Goller         | May 2, 1950   |
| 2,703,298 | Branson et al. | Mar. 1, 1955  |

#### OTHER REFERENCES

Uhlig: Trans. A.S.M., vol. 30, pages 949-980, especially pages 947, 954, 958, 978. 1942.